

## UNITED STATES PATENT OFFICE

2,336,252

## TREATMENT OF COTTON

Florence E. Hooper, Yonkers, N. Y., assignor to  
The Chemical Foundation, Incorporated, a corporation of Delaware

No Drawing. Application January 6, 1940,  
Serial No. 312,687

11 Claims. (Cl. 260—212)

This invention relates to the treatment of cotton, more particularly to a novel bacterial treatment of cotton as a result of which the cotton is improved for subsequent treatment.

In the past it has been observed that rayons, produced wholly or in part from cotton, sometimes contain specific inhomogeneities which seriously detract from the value of the product. For example, many times in a given production of cuprammonium silk it will be found that the extruded thread has segregated small areas which are non-receptive to a dye. Such a differential dyeing ruins the thread for many purposes.

It has been ascertained that this and kindred difficulties may be largely due to the cuticle of the cotton fiber which is not removed during the purification. While the cotton fiber consists essentially of ellipsoidal, crystalline cellulose particles dispersed in a continuous phase of a cementing material, it does also contain, in the limiting membrane, a non-cellulosic material of a waxy nature. This material, sometimes referred to in the literature as cutocellulose, is very small in amount but is of such a resistant or refractory character that in many circumstances it passes unchanged through the purification treatments and appears in the final product. Its presence is distinctly disadvantageous not only because it is a positive inhomogeneity and may well spoil a dyed thread or sheet, but also because it appears to inhibit the dispersion of the cellulose particles in dispersing solutions such as cuprammonium hydroxide.

While this undesired constituent could be removed by decomposing it with chemical reagents, a drawback of such a method, however, would be a concomitant and undesired degradation of the other constituents of the fiber. The ideal method of removal of this cuticle material is one which is directly selective and which removes such material without undesired change or modification of the other components of the cotton fiber.

After extensive experimentation, it has been found that this undesired non-cellulosic waxy constituent may selectively be removed by a controlled bacterial treatment and without any substantial action on the other constituents of the fiber. With such a treatment, an improved raw material for rayon production is made available. Furthermore, another important and advantageous concomitant of the novel treatment is that fibers so treated disperse much more readily and

uniformly in typical dispersing solutions than do untreated fibers.

Preliminary investigations conducted to establish the best commercial method conclusively show that certain aerobic cellulose-decomposing bacteria from the soil, when properly cultured on raw cotton, act in two more or less definite sequential stages. The bacteria first act on the cuticle of the cotton to directly decompose it, and then the bacteria more slowly disintegrate the fiber itself. It is particularly to be observed, therefore, that the present invention involves not only a specific bacterial action but that it also involves a distinct specificity with respect to the time of the action. For example, cellulosic-decomposing bacteria when cultured on raw cotton in the presence of inorganic salts and at a temperature of 25° to 30° C. first act on the cuticle. If such inoculated fibers are removed from the culture at the end of about five days and are washed, it is found that the cuticle is completely removed but the fibers are otherwise intact. It is particularly interesting to observe that the viscosity of the treated fibers when dispersed in cuprammonium hydroxide remains unchanged. The fibers treated by this bacterial method, however, disperse much more rapidly and uniformly in cuprammonium hydroxide and xanthate solutions than do the untreated fibers.

In the course of experimentation, it was found that a large number of cellulose-decomposing bacteria are operative in the process. These bacteria, which are notably difficult of classification, include members of the cellulose-decomposing genera of the Pseudomonadaceae, namely, Cellvibrio and Cellfalciculus, as well as members of the genus Bacteriaceae, as for example Cellulomonas.

In carrying out the process, a quantity of cotton is placed in a nutrient salt solution, then sterilized, as by autoclaving at elevated temperatures, and inoculated with a pure culture of the micro-organism. At the end of the period required to remove the cuticle the bacteria are killed, as for example by autoclaving or by heating for 10 minutes at a temperature of approximately 75° C. The treated cotton may then be washed, filtered and air-dried. While it has been determined that a definite time period must be allowed for the selective action of the bacteria on the cuticle, there is, of course, no abrupt or sharp demarcation of the cessation of the action on the cuticle and the institution of bacterial action on the fiber per se. It has been found, as an operative fact, that a period of five

days is amply sufficient to insure the destruction of the cuticle and without any substantial action on the other constituents.

In commercial production the bacterial treatment may be conducted at any stage which most readily conforms to the requirement of a particular plant or process. Other things being equal, it is preferable to effect the selective removal of the undesired cuticle-like constituents of the raw cotton prior to subsequent treatments, such as treatments with caustic for the formation of alkali cellulose. In any event, due to the noted fact that the treatment does improve the dispersibility of the cellulose of the fiber, it is preferable to effect the selective bacterial treatment prior to the dispersion of the cellulose in a dispersing medium such as cuprammonium hydroxide or xanthate solutions.

Improved material for cuprammonium rayons may be produced under the present invention by first subjecting cotton linters to the described bacterial treatment. The treated fibers may then be given a pretreatment in sodium hydroxide, in the known manner and then dispersed in cuprammonium hydroxide to form a spinning solution. With such a treatment it is found that the cellulose dispersed very readily in the cuprammonium hydroxide and the regenerated fiber or sheet produced is characterized by a greatly increased uniformity in dye acceptance.

Similarly, improved material for acetate silks may be produced by subjecting the cellulosic starting material, such as cotton linters, to the improved selective bacterial action. Thereafter the fibers may be treated with the known mixture of acetic anhydride, glacial acetic acid and sulphur dioxide. Floccules produced by the addition of water may be dissolved in acetone to form a spinning solution and the solution is extruded into the desired form in the known manner.

In the production of viscose rayons it is preferable to first subject any cuticle-containing raw material to the described bacterial action prior to treatment with the 18% caustic solution, i. e., prior to the formation of the alkali cellulose. It has been found, as noted, that this bacterial pretreatment not only insures the production of an improved fiber but also greatly facilitates the dispersion of the alkali cellulose in the xanthate solution.

It will thus be appreciated that the method herein described is available for improvement in any technological field where the cotton fiber is used in the original or the regenerated, reconstituted or derivative form. As noted hereinbefore, selective removal of the cuticle insures a more uniform dyeing due to the fact that the waxy dye-resistant material is removed. While the process is particularly valuable for the treatment of cotton fibers entering into rayon production, it is also available for the treatment of cotton, as such, which is subsequently utilized in the production of cotton fabrics. It will be understood, therefore, that the invention resides in the broad concept of the selective bacterial removal of those constituents which are comprised in the cuticle phase of the cotton fiber and in other cellulosic products in which a chemical phase equivalent to the cuticle of the cotton fiber is involved. The new method may thus be used with advantage in the production of viscose rayon, acetate rayon, cellulose ethers, such as ethyl cellulose, and esters, such as gun cotton cellulose nitrate and the like.

I claim:

1. As a new product, cotton fiber, characterized by a ready dispersibility in cellulose dispersion agents, which has been subjected to the action of aerobic cellulose-decomposing bacteria for a time sufficiently prolonged to decompose the cuticle but without substantial decomposition of the cellulose.
2. A rayon, characterized by a highly uniform dye acceptability, produced at least in part from cotton fibers which have been subjected for a limited period of time to the action of aerobic cellulose-decomposing bacteria.
3. A rayon, characterized by a highly uniform dye acceptability produced at least in part from cotton fibers which have been subjected for a limited period of time to the action of a Pseudomonadaceae to decompose the cuticle of the fibers without substantial decomposition of the cellulose.
4. A method of producing dispersions of cotton which comprises subjecting the cotton to the action of an aerobic cellulose-decomposing bacteria for a period of approximately five days, treating the cotton to inactivate and remove the bacteria, and subsequently dispersing the treated material in a cellulose-dispersing solution.
5. A method of producing readily dispersible alkali cellulose which comprises treating cotton with an aerobic cellulose-decomposing bacteria for a period of time sufficiently prolonged to destroy the cuticle of the cotton, removing the bacteria and its decomposition products and treating the cotton with sodium hydroxide of substantially 18% concentration.
6. A method of producing readily dispersible alkali cellulose which comprises treating cuticle-containing cellulose with an aerobic cellulose-decomposing bacteria for a period of time sufficiently prolonged to destroy the cuticle but without any substantial decomposition of the cellulose, removing the bacteria and its decomposition products and treating the cellulosic material with sodium hydroxide of substantially 18% concentration.
7. A method of purifying cotton which comprises inoculating cotton in the presence of a nutrient salt solution with a culture of a Pseudomonadaceae, maintaining the solution at a temperature of the order of 25° C. for a period approximating five days, inactivating the bacteria, and removing the bacteria and its decomposition products from the cotton.
8. A method of purifying cotton which comprises inoculating cotton in the presence of a nutrient salt solution with a culture of a cellulose-decomposing Bacteriaceae, maintaining the solution at a temperature of the order of 25° C. for a period approximating five days, inactivating the bacteria, and removing the bacteria and its decomposition products from the cotton.
9. A method of purifying cotton which comprises sterilizing cotton in the presence of a nutrient salt solution, inoculating the cotton with a culture of *Cellvibrio*, maintaining the mass at a temperature of substantially 25° C. for a period of from four to six days, heating the mass to a temperature sufficiently high to inactivate the bacteria and separating the bacteria and its decomposition products from the cotton.
10. A method of purifying cotton which comprises sterilizing cotton in the presence of a nutrient salt solution, inoculating the cotton with a culture of *Cellfaliculiclo*, maintaining the mass

at a temperature of substantially 25° C. for a period of from four to six days, heating the mass to a temperature sufficiently high to inactivate the bacteria and separating the bacteria and its decomposition products from the cotton.

11. A method of purifying cotton which comprises sterilizing cotton in the presence of a nutrient salt solution, inoculating the cotton

5 with a culture of Cellulomonas, maintaining the mass at a temperature of substantially 25° C. for a period of from four to six days, heating the mass to a temperature sufficiently high to inactivate the bacteria and separating the bacteria and its decomposition products from the cotton.

FLORENCE E. HOOPER.